

April 3, 1973

J. Y. RIEDEL

3,725,050

COLD WORK DIE STEEL

Filed March 2, 1970

*Fig. 1*



*Fig. 2*



*INVENTOR*  
*John Y. Riedel*

## 1

3,725,050

### COLD WORK DIE STEEL

John Y. Riedel, Bethlehem, Pa., assignor to  
Bethlehem Steel Corporation

Filed Mar. 2, 1970, Ser. No. 15,482  
Int. Cl. C22c 39/14

U.S. CL. 75—126

2 Claims

#### ABSTRACT OF THE DISCLOSURE

A malleable cold work die steel containing large amounts of titanium carbides in a matrix of tempered martensite. 10

#### BACKGROUND OF THE INVENTION

This invention relates to tool steels, and more particularly to cold work die steels.

Cold work die steels are commonly used in apparatus for forming sheet steel. In many forming operations, particularly where the deformation is severe, the oxide layer at the surface of the sheet is broken up as the sheet is being deformed. The high pressures accompanying deformation may cause particles of the metal formerly underlying this oxide layer to weld to the die wall. As a result of this welding action, during subsequent deformations one of two things will happen. The welded particle may be pulled off the die wall along with a small piece of the die itself. This constitutes wear of the die wall. Alternatively, the welded particle may remain on the die wall and act as a cutting tool on the workpiece. This problem of metal pick-up by the die, referred to in the art as galling, is an important factor in die wear.

Another important factor in die wear is abrasion resulting from small particles of material interposed between the rubbing surfaces of the die and the workpiece.

Resistance to galling and abrasion are not the only factors to be considered in the selection of a cold work die steel. Other factors include toughness, machinability and grindability.

In the past, steels were known which were characterized by the combination of both a fairly good resistance to galling and abrasion as well as good toughness, machinability and grindability. An example of such a steel is as follows:

|                     | C    | Mn   | Si   | Cr   | V    | Mo   |
|---------------------|------|------|------|------|------|------|
| Weight percent..... | 1.00 | 0.60 | 0.25 | 5.00 | 0.25 | 1.00 |

Better wear resistance could be obtained by increasing the amount of carbon and carbide-forming elements in the steel. This however, resulted in a substantial decrease in toughness, machinability and grindability. Examples of such steels are as follows:

| Steel                   | C    | Mn   | Si   | Cr    | V    | Mo    | W     |
|-------------------------|------|------|------|-------|------|-------|-------|
| (A) Weight percent..... | 1.50 | 0.30 | 0.25 | 12.00 | 0.60 | 0.80  | ..... |
| (B) Weight percent..... | 2.4  | 0.40 | 0.40 | 12.50 | 4.00 | ..... | 1.00  |

It is an object of this invention to provide a cold work die steel having the combination of extremely good resistance to galling and abrasion as well as very good toughness, machinability and grindability.

#### SUMMARY OF THE INVENTION

I have discovered that the foregoing object can be obtained by providing a steel having relatively high amounts of titanium in combination with relatively low amounts of chromium. The titanium combines with the carbon in the steel to form extremely hard titanium carbides which impart high wear resistance to the steel. By limiting the chromium content of the steel, the amount of chromium carbides which form is limited. Inasmuch as carbides de-

## 2

tract from toughness, limiting the chromium content is thus conducive to good toughness.

#### BRIEF DESCRIPTION OF THE DRAWINGS

5 FIG. 1 is a photomicrograph of a typical prior art cold work die steel.

FIG. 2 is a photomicrograph of an example of the steel of the invention.

#### DESCRIPTION OF THE PREFERRED EMBODIMENT

Broadly, the steels of the invention consist essentially of 0.85 to 1.50 wt. percent carbon, 0.20 to 2.00 wt. percent manganese, 0.80 to 2.00 wt. percent titanium, 3.50 15 wt. percent max. chromium, 2.00 wt. percent max. molybdenum, balance essentially iron. In addition, for reasons to be explained hereinafter, the wt. percent carbon must be equal to at least 0.65 plus 1/4 times the titanium. The steel may also contain up to 1.20 wt. percent tungsten. By 20 "balance essentially iron," I do not wish to exclude residual impurities and incidental elements which may be present in amounts which do not substantially detract from the novel properties of the steel. Preferably, the aluminum content should be limited to 0.10 wt. percent max., the silicon to 0.40 wt. percent max., and the nitrogen to 0.010 25 wt. percent max.

The reasons for the above range limitations are as follows. Inasmuch as the amount of carbon desired in the steel depends upon the titanium content thereof, titanium 30 will be discussed first. The steel should contain a minimum of 0.80 wt. percent titanium to insure that a large amount of titanium carbides form. Increasing the amounts of titanium and carbon in the steel results in an increasing volume percentage of titanium carbides and improved 35 wear resistance. However, the toughness, machinability and grindability decrease as the volume percentage of titanium carbides increases. An excellent combination of these properties can be obtained if the titanium is limited to 2.00 wt. percent max.

The steel should contain a minimum of about 0.55 wt. percent carbon to insure that the as-quenched hardness of the steel is at least 64 Rockwell C. Additional carbon is necessary for combining with the titanium to form titanium carbides. This amount of carbon is equal to, by weight, 45 1/4 the amount of titanium. An additional 0.10 wt. percent carbon has been found necessary to insure a minimum hardness of 60 Rockwell C after tempering the as-quenched roll at 300 to 400° F. Thus, the total wt. percent of carbon in the steel should be equal to at least 50 0.65 plus 1/4 times the titanium. Since the minimum titanium in the steel is 0.80 wt. percent, the minimum carbon is 0.85 wt. percent.

Increasing the volume percentage of carbides in the steel decreases the toughness thereof. For this reason, the 55 carbon content of the steel should be limited to 1.50 wt. percent max.

A minimum of about 0.20 wt. percent manganese is necessary to prevent hot-shortness, while manganese in excess of about 2.00 wt. percent imparts excessive brittleness to the steel. Chromium and molybdenum are included in the steel for the purpose of hardenability. The upper limits therefor, set forth above, are necessary to prevent the steel from becoming unduly brittle due to excessive carbide formation.

65 Tungsten may also be present in the steel. This element substitutes for a portion of the titanium in the titanium carbides, thus increasing the volume percentage of the titanium carbides in the steel. Tungsten, however, also substitutes for a portion of the chromium in the chromium carbides, thus increasing the volume percentage of the chromium carbides in the steel. As above noted, increasing 70 the volume percentage of carbides decreases the

3 toughness of the steel. For this reason, the tungsten must be limited to about 1.20 wt. percent max.

|                     | C    | Mn   | Ti   | W    | Cr   | Mo   | Al    | Si   | N     | P     | S     |
|---------------------|------|------|------|------|------|------|-------|------|-------|-------|-------|
| Weight percent..... | 0.99 | 0.69 | 0.96 | 0.84 | 3.01 | 1.05 | 0.030 | 0.35 | 0.008 | 0.003 | 0.007 |

The aluminum and silicon in the steel are preferably limited to 0.10 wt. percent max. and 0.40 wt. percent max., respectively. The reason for this is that both of these elements are strong graphitizers. The formation of graphite reduces the amount of carbon available for hardening and also reduces toughness. In addition, silicon contributes to decarburization during heating.

Titanium carbide has been found to be much harder than titanium nitride. Hence, for a given titanium content, it is desirable to maximize the amount of titanium carbide and minimize the amount of titanium nitride in the steel. Limiting the nitrogen content of the steel to 0.010 wt. percent max. results in the formation of a minimum amount of titanium nitrides.

For an optimum combination of properties, the following ranges of elements are preferred:

|                     | C         | Mn      | Ti        | W         | Cr        | Mo        | Al        | Si        | N     |
|---------------------|-----------|---------|-----------|-----------|-----------|-----------|-----------|-----------|-------|
| Weight percent..... | 0.90-1.10 | .40-.80 | 0.80-1.50 | 0.90-1.20 | 2.75-3.25 | 0.90-1.25 | 0.01-0.03 | 0.15-0.40 | 0.010 |

FIGS. 1 and 2 provide a visual comparison of the microstructures of a typical prior art cold work die steel with a steel of the invention. The compositions of these steels are as follows:

| Steel                                 | C    | Mn   | Si   | Cr  | V    | Mo   | W     | Ti    | N     |
|---------------------------------------|------|------|------|-----|------|------|-------|-------|-------|
| Prior art<br>(weight<br>percent)..... | 1.02 | 0.59 | 0.29 | 5.2 | 0.24 | 1.02 | ..... | ..... | Res.  |
| Invention<br>(weight<br>percent)..... | 1.00 | 0.60 | 0.40 | 3.0 | 0.25 | 1.0  | 1.00  | 1.00  | 0.005 |

Both figures are photomicrographs, at 500 magnifications, after a picral etch. In FIG. 1, the specimen was austenitized at 1775° F., air quenched, and tempered at 400° F. for 4 hours. The microstructure consisted of  $M_{23}C_6$ — and  $M_7C_3$ — type carbides in a matrix of tempered martensite.

In FIG. 2, the specimen was austenitized at 1750° F. and oil quenched. The large angular particles are titanium carbides, while the small rounded particles are  $M_{23}C_6$ — type carbides. The matrix is martensite.

It is clear from a comparison of FIGS. 1 and 2 that the microstructure of the steels of the invention differs substantially from that of the prior art steel shown. The titanium carbides shown in FIG. 2 are much harder than both the  $M_{23}C_6$ — type and the  $M_7C_3$ — type carbides. Said titanium carbides impart wear-resistance to the steel.

Steels of the foregoing compositions may be produced in the usual manner. For example, a melt of such a steel may be prepared in an electric furnace and teemed into ingot molds. Following solidification, the ingots are either hot rolled into billets or press forged into other desired shapes. The resultant product is subsequently annealed, surface conditioned, and formed into the desired product. For example, a billet may be hot rolled into bars. The bars are annealed, rough-machined into a tool, quenched and tempered, and finish-ground.

As a specific example of the invention, an experimental 500 lbs. heat of steel was melted in an induction furnace,

cast into a 9 inch square ingot mold and hot topped. The composition of the steel was as follows:

The ingot was heated to about 2050° F., forged into a 6 inch square billet, and cooled slowly to room temperature. The billet was then annealed by a process comprising heating to 1450° F., holding at said temperature for 10 hours, cooling to 900° F. at a rate of 30° F./hour, and air cooling to room temperature. The longitudinal surface of the billet was then ground to remove defects therefrom.

15 The billet was subsequently reheated to about 2050° F., forged into a bar 2 1/4 x 3 3/4 x 36 inches, and cooled slowly to room temperature. Next, the bar was annealed by a process comprising heating to 1600° F., holding at said temperature for 8 hours, cooling to 900° F. at a rate of 30° F./hour, and air cooling to room temperature. The bar was then rough-machined into a die.

The rough-machined die was heat treated by a process

comprising preheating to 1200° F., heating to 1775° F., holding the die at 1775° F. for 1 hour per inch of greatest cross-section, and quenching by air cooling to room temperature. The quenched die was then tempered by holding it at 350 to 400° F. for 2 hours per inch of greatest cross-section. Following tempering, the die was finish-machined and tested for defects.

30 The die was used in a die for punching sheet steel. The service life of the piece was found to be superior to that of steels containing relatively large amounts of chromium and carbon, e.g. steels such as the type above designated as "A" and "B."

I claim:

40 1. A malleable steel consisting essentially of 0.90 to 1.10 wt. percent carbon, 0.40 to 0.80 wt. percent manganese, 0.80 to 1.50 wt. percent titanium, 0.90 to 1.20 wt. percent tungsten, 2.75 to 3.25 wt. percent chromium, 0.90 to 1.25 wt. percent molybdenum, balance essentially iron, said steel being adapted to be heat treated to have a microstructure consisting essentially of undissolved carbides in a matrix of tempered martensite.

45 2. A cold work die formed of the steel of claim 1.

#### References Cited

##### UNITED STATES PATENTS

|              |         |           |          |
|--------------|---------|-----------|----------|
| 1,839,157    | 12/1931 | Mathesius | 75—126 D |
| 2,362,046    | 11/1944 | Bonte     | 75—123 M |
| 55 2,665,205 | 1/1954  | Klaybor   | 75—126 E |
| 2,132,877    | 10/1938 | Naumann   | 75—126 C |
| 3,330,651    | 7/1967  | Younkin   | 75—123 M |
| 1,981,898    | 11/1934 | Boegehold | 75—126 D |
| 2,923,619    | 2/1960  | Culp      | 75—126 C |
| 60 2,968,549 | 1/1961  | Brady     | 75—126 C |
| 3,044,872    | 7/1962  | Hayes     | 75—126 D |
| 2,115,465    | 4/1938  | Merten    | 75—126 C |

HYLAND BIZOT, Primary Examiner